

Sept. 25, 1928.

1,685,281

W. F. FOX

PRODUCTION OF COLORED PHOTOGRAPHS

Filed June 22, 1920

*Fig. 1,*



*Fig. 2,*



*Fig. 3,*



*Fig. 4,*



*Fig. 5. 4*



Inventor  
William F. Fox

By his Attorney

*J. Edmonds*

Patented Sept. 25, 1928.

1,685,281

# UNITED STATES PATENT OFFICE.

WILLIAM FRANCIS FOX, OF NEW YORK, N. Y., ASSIGNOR TO NATURAL COLOR PICTURES COMPANY, INC., OF NEW YORK, N. Y., A CORPORATION OF DELAWARE.

## PRODUCTION OF COLORED PHOTOGRAPHS.

Application filed June 22, 1920. Serial No. 390,901.

My invention relates to a process for the production of positives in color, applicable to cinematography or still photography. It also relates to a novel form of colored photographs or series of such colored photographs for use in cinematography, or projection, as articles of manufacture.

In accordance with my invention a base formed of transparent or translucent material is coated with a sensitive emulsion, which should be thicker than the usual emulsion used in black and white photography. Images in alignment with each other are printed on this single coating of emulsion, one of such images being formed on or adjacent to the rear surface of the emulsion, the other image being formed on the front or outer surface of the emulsion. These images being suitably colored there will result a composite image which may be in approximately natural colors, formed by a pair of aligned images carried by a single coating of gelatin or other emulsion material upon one side of a suitable light-transmissive base. The emulsion may contain a coloring material, preferably a water-soluble yellow dye, adapted to prevent the actinic light-rays from penetrating entirely through the emulsion. The image which is formed on or adjacent to the under surface of the emulsion coating is printed through the base, the soluble dye which was carried by the emulsion being subsequently removed.

In my application entitled "Improvements in color photography," Serial Number 390,902, filed on even date herewith, the process briefly referred to above, is claimed in its broad aspect and the product formed thereby is also broadly claimed. In the present application a process will be claimed which is specifically different from that specifically described and claimed in my said co-pending application. I will also claim herein a form of product which is different from that specifically described in my said co-pending application.

In my said co-pending application positive images are printed in alignment on the upper and under surfaces of the single emulsion coating in alignment with each other, which images may be printed from negatives of the same object taken through complementary color screens. The film is toned, or mordanted and dyed to a color suitable for the under image, after which the clear gelatin is

hardened or otherwise treated to cause the same to resist rapid penetration, by a subsequent toning solution. The top image is then turned over to the complementary color by a suitable toning operation, the treatment to which the clear gelatin was submitted preventing penetration of the same by the toning solution.

In the invention to be described in the present application, the image which is printed through the base is a positive from one of the two negatives referred to. The image which is printed in alignment therewith on the upper surface of the emulsion is, however, a negative image, corresponding to the other of the two negatives taken through the complementary color screens. The film is then toned to a color appropriate to the under image and the gelatin is at the same time hardened in proportion to the amount of tone. The film is now subjected to the action of an acid dye bath, of a color complementary to that which was produced by the toning. This will act most vigorously on the soft portions of the film and less vigorously on the hardened portions. This dyeing operation will color the parts of the top image which were white, and will change the parts of the top image which were of the color of the toning bath, to white. The result of this treatment will be to change the top image to a positive representation of the color elements which passed through the color screen from which the negative corresponding to the top image was taken.

Attention is hereby directed to the accompanying drawings forming part of this application and illustrating diagrammatically my improved process. In the drawings Fig. 1 represents a portion of a single coated film or base having a positive image formed on the under side of the emulsion coating, the latter being shown partly separated from the base, for purposes of illustration, Fig. 2 shows the same portion of film within a negative image formed on the upper surface of the emulsion in registry with the under image, Fig. 3 represents the same portion of film with designation of the first coloring step and the hardening of the emulsion, Fig. 4 represents the same portion of film with designation thereon of the final color step, and Fig. 5 shows the same portion of film with the negative image formed on the upper surface of the emulsion through a line screen.

Proceeding now to a more detailed description of my present process, the latter may be referred to as a two-color process in which the negatives are made in the usual way, one being photographed through a red screen and the other through a green screen. It should be understood that by a "red" screen I intend to include screens of any color passing a maximum quantity of red rays and by a "green" screen I intend to include screens of any color passing a maximum quantity of green or blue rays, whichever may be complementary to the "red" screen. The two screens are, in fact, complementary, the term "red" and "green" being used to readily distinguish the one from the other.

Having obtained the negatives, the positives may be formed in the following manner: A transparent or translucent base 1 is coated 20 with a suitable sensitive emulsion 3 of any usual character suitable for color photography, on one side of the base only. The base may be formed of the usual pyroxylin film stock used in cinematography, or the like, or 25 glass if desired, for still photography. A dye is incorporated in the emulsion suitable to prevent actinic light-rays penetrating through the body of the emulsion when the images are printed from opposite sides of the film. 30 I have found a yellow dye is well adapted for this purpose, tartrazine being particularly suitable. This dye is water-soluble so that in the operations of developing and treating the emulsion it will wash out of the gelatin, 35 or other emulsion material used. This coating of emulsion, as stated above, is somewhat thicker than the usual emulsion used in black and white photography since a portion of the same must separate the two images in 40 alignment.

A print is made from one of the negatives, the image being printed through the light-transmissive-base 1, upon the under side 2 of the emulsion coating 3, so that the impressed 45 image does not penetrate through to the top or front side 4 of the emulsion. This printed image when developed will be a positive representation 5 of certain color values of the picture. As an example of my process it may 50 be assumed that this print is made from the negative taken through the red filter so that the printed image referred to, when developed, will be a positive representation of the green values of the picture.

Printed directly over and in alignment with 55 this image, but from the front or top side of the emulsion will be a negative representation 6 of the red values of the picture, in the example referred to. This top negative image 60 6 will be obtained from a positive print which may be made in the ordinary way, obtained from the negative taken through the green filter, the image on the emulsion being printed from this positive.

65 The two impressed images 5 and 6 are now

developed in the ordinary developer, fixed and washed. If the print is now examined it will be found to contain one positive image of the green color values and one negative image of the red color values.

The print is now toned to a suitable color corresponding to the color values of the positive print as at 7 (see Fig. 3). Any toning bath may be used which will, while toning the images, so harden the gelatin as to prevent, to a varying extent depending on the amount of silver originally present in the image, the penetration of an acid dye. A suitable toning bath is made up of

|                         |            |
|-------------------------|------------|
| Vanadium chloride       | 20 grains  |
| Ferric ammonium oxalate | 10 grains  |
| Ferric chloride         | 10 grains  |
| Potassium ferricyanide  | 20 grains  |
| Glacial acetic acid     | 10 minims  |
| Oxalic acid             | 100 grains |

Sufficient water to make total composition 100 ounces.

After toning, as described, the film is now immersed in a suitable clearing bath, which may be a sodium thiosulphate bath, and is then washed and dried. We now have a film the gelatin coating of which contains two images 5 and 6, both colored green as at 7; the yellow dye having been previously washed out of the gelatin. The bottom image, the one that was printed through the base, will remain green in the finished print, but the top image must be changed over to a red color as at 8 (see Fig. 4). The top image is a negative, so that the parts of the original object photographed which were white are green in this toned image, and the parts which were red in the original object are clear gelatin. In toning this negative image to a green color the 95 gelatin was hardened pro rata to the amount of toning so that in the clear portions of the film the gelatin is soft, and in the parts, where there is a large amount of green color the gelatin is hard. It is well known that if certain 100 green tones are stained with a red dye, the dye will enter the film to a limited extent, changing over the color of the tone practically to white. This can readily be done providing 105 the printing and developing of the original image has not been carried too far since if the tone is too heavy the dye will not penetrate the film at all.

In practicing my invention the toning is carried out to such an extent as to allow as nearly a perfect white as possible with the maximum quantity of red dye in the clear portion of the gelatin. The film now being immersed in a suitable acid red dyeing bath, the dye will act most vigorously on the soft portions of the film and less vigorously on the hardened portions. This will convert the negative image of the red impressions to a positive image of the red as seen in the original object photographed. The parts of the 110

upper image which were of a green color will now be white or approximately so and the parts of the image which were white will be of a full red. Thus are obtained a red and a green image in the one coat of emulsion material, as the under image will not be affected by the dye, the top image preventing penetration of the dye to any parts of the under image where the dye should not go.

10 Various acid red dyes may be used in practicing the process.

Full reds will easily be obtained in the process described since the clear gelatin in the two images will not be hardened, thus allowing the dye to penetrate to the full thickness of the gelatin. Greens will be obtained by the green in the under image being seen through the white image of the top print. Whites will be clear gelatin in the under image protected by the tone in the top image, which tone has been converted to white by action of the dye. Blacks will be obtained by the under image having a full green, while the top image has an aligned portion of surface in which the clear gelatin has been dyed to a full red and so on through the scale of colors obtainable.

In printing the top image on the emulsion it may be found better to use a line screen, or a screen composed of dots, in order to obtain a better quality of white. This screen may be similar to the ones used in half tone process work and will split up the top image as shown at 9 (see Fig. 5) so that the dye will be better able to combine with the green tone in order to form white. This line screen may be interposed in any position between the printing positive, from which the negative is printed on the top of the emulsion, and the emulsion, so that the resultant image will be broken up the better to allow the action of the dye. While the use of such a screen may sometimes be of advantage in making the top image, it will not be necessary in printing the under image.

45 To obtain the positive for printing the top image, many methods may be employed. The simplest way is to make a positive by contact printing and use this for printing the top image. Another method is to chemically reverse the green negative before fixing the same in one of the many well known reversing baths such as one containing potassium permanganate and sulphuric acid.

In cinematography, where a continuous series of pictures is required to be printed, and shrinkage of the negative is to be taken into consideration, a so-called "dupe" or secondary printing negative may be made, consisting of an alternate negative image and positive image. A negative image of the object photographed through the red filter and a positive image of the object photographed through the green filter would then appear side by side on the same length of the film, or alternately in a straight line sequence, if de-

sired. This would prevent the chance of error due to shrinkage of a separate positive or negative.

In cinematography, if the red and green pictures alternate in straight line sequence in the original negative, a special form of printing machine will have to be used in order to obtain the proper sequence of the prints with all the red prints in straight line sequence on one side of the emulsion coating and all of the green prints in alignment therewith on the opposite side of the emulsion coating. Suitable apparatus may be obtained for this purpose and is, of course, no part of my present invention. In taking the original negatives, however, two negative strips may be taken side by side one through a green filter and one through a red filter and one of these strips converted to a positive after which the two separate strips may be used for printing. In this case a specially designed printer would not be required provided that the mechanism of the printer were accurate.

The film should be immersed in a suitable acid red dye bath, as stated, until the whites show up pure white after which the film may be rinsed in clear water and dried. It is then ready for projection.

It should be understood that the description given above, in which the under print is made from the negative taken through the red filter and the upper print corresponds to the negative taken through the green filter, is given by way of example and not by way of limitation of my invention. This process may be reversed, the under print being made from the negative taken through the green filter and the film toned in a suitable red toning bath after which the upper image is printed from a positive made from a negative taken through the red filter, a suitable green acid dye being then used for the final coloring step.

What I claim is:

1. A photographic process comprising, printing a positive image and a negative image of the same object in alignment in a single coating of sensitive emulsion on one side of a suitable base, with unaffected emulsion separating said images, said positive image being undermost, toning both images one color and hardening the emulsion material in proportion to the amount of tone, and dyeing the film with a dye of a second color, adapted to act most vigorously on the soft portions of the film.

2. A photographic process comprising, printing a positive image and a negative image of the same object in alignment in a single coating of sensitive emulsion on one side of a suitable base, with unaffected emulsion separating said images, said positive image being undermost, said positive print being made from a negative from which certain color sensations are omitted and said

negative print having complementary color sensations omitted therefrom, toning both images a color corresponding to the color values of said positive print, and hardening the emulsion material in proportion to the amount of tone, and dyeing the film with an acid dye of a color complementary to that imparted by the toning, said dye being adapted to act most vigorously on the unhardened portions of the film.

3. A photographic process, comprising, printing a positive image and a negative image of the same object in alignment in a single coating of sensitive emulsion on one side of a suitable base, with unaffected emulsion separating said images, said positive image being undermost, said positive print being made from a negative from which green color sensations are omitted and said negative print having red color sensations omitted therefrom, toning both images green, and hardening the emulsion material in proportion to the amount of tone, and dyeing the film with a red acid dye, said dye acting most vigorously on the unhardened portions of the film, and converting the parts of the upper image which were green to white.

4. A photographic process, comprising printing a positive image through a light transmissive base on the under surface of a coat of sensitive emulsion on the other side of the base, from a negative from which certain color sensations have been omitted, the emulsion being so treated as to prevent the actinic light rays from penetrating entirely through the emulsion, printing a negative image of the same object, from which color sensations are omitted, different from those omitted from the negative first mentioned, on the upper surface of said emulsion coating, in alignment with said positive image, developing, fixing, toning the film to a desired color, and hardening the emulsion material in proportion to the amount of tone, and dyeing the film with a dye of a second color,

adapted to act most vigorously on the soft portions of the film.

5. A photographic process, comprising printing a positive image through a light transmissive base on the under surface of a coat of sensitive emulsion on the other side of the base, from a negative from which certain color sensations have been omitted, the emulsion being so treated as to prevent the actinic light rays from penetrating entirely through the emulsion, printing a negative image of the same object, from which color sensations are omitted, complementary to those omitted from the negative first mentioned, on the upper surface of said emulsion coating, in alignment with said positive image, developing, fixing, toning the film to a color corresponding to the color values of said positive print and hardening the emulsion material in proportion to the amount of tone and dyeing the film with an acid dye of a color complementary to that imparted by the toning, said dye being adapted to act most vigorously on the unhardened portions of the film.

6. As a new article of manufacture, a light transmissive base having a coating of emulsion material on one side, with two images of the same object formed therein in alignment, one of the same being a negative image, and the other formed on the under surface of said coating, being a positive image.

7. As a new article of manufacture, a light-transmissive base having a coating of emulsion material on one side, with two images of the same object formed therein in alignment, one of the same being a toned image, formed on the under surface of said coating, representing certain color values of the object photographed, and the other being a dyed image, representing complementary color values of the object photographed.

This specification signed and witnessed this 1st day of June, 1920.

WILLIAM FRANCIS FOX.